

3,189,447  
ELECTROPHOTOGRAPHIC MATERIAL  
AND METHOD

Wilhelm Neugebauer, Martha Tomanek, and Hans Behmenburg, all of Wiesbaden-Biebrich, Germany, assignors, by mesne assignments, to Azoplate Corporation, Murray Hill, N.J.

No Drawing. Filed May 29, 1957, Ser. No. 662,319  
Claims priority, application Germany, June 4, 1956,  
K 29,014

41 Claims. (Cl. 96—1)

This invention relates to photographic reproduction and more particularly to electro-photographic processes, namely processes in which an electrostatic latent image is produced by utilising the property of photoconduction (i.e., a variable conductivity dependent on the intensity of illumination). The electrostatic latent image may be produced in a conventional exposure operation, for example by means of a lens-projected image or by contact-printing techniques, whereby a non-visible electrostatic charge pattern (the so-called electrostatic latent image) is created on a surface, in which pattern the charge density at any point is related to the intensity of illumination obtaining at the point during the exposure. The latent image may be developed—i.e., rendered visible—by means of an electroscopic powder, such as a coloured synthetic resin powder, and the resulting visible image may be fixed by rendering the powder permanently adherent to a support on which the image is desired, for example in suitable cases by heating to soften or melt the powder particles and/or the surface of the image support, or by application of an electric field, or with volatile solvents.

In electro-photographic processes the electrostatic latent image is commonly formed on the surface of a photoconductive insulating layer carried on a support. For example, material comprising such support and photoconductive layer may be sensitized by applying a uniform surface charge to the free surface of the photoconductive layer, for example, by means of a corona discharge, which charge is retained owing to the substantial insulating character, i.e., the low conductivity, of the layer in the dark. On exposure as described above, the photoconductive property of the layer causes the conductivity to increase in the illuminated areas to an extent which is proportional to the intensity of illumination. This results in a leakage of the surface charge in the illuminated areas while the charge in the unilluminated areas remains. This is what constitutes the aforementioned charge pattern or electrostatic latent image.

Electro-photographic processes have become of increasing importance in recent years, especially in connection with office duplicating processes where, offering as they do a wholly dry copying process, they are usually preferable to other types of photo-copying. Consequently, there has been much interest aroused and much effort has been made to obtain suitable materials for making the support and photoconductive insulating layers used in such processes.

Various proposals in regard to such materials have been made in an effort to fulfill modern requirements with regard to range of use, reliability, simplicity in handling, potential light sensitivity and storage qualities. Among those photoconductive substances used hitherto, selenium has been the most notable, although many other materials have also been used. However, all these prior materials had various disadvantages which have now been overcome by the present invention.

Generally described, the present invention provides a material for use in electrophotographic processes, which is capable of being rendered light sensitive by applying an electrostatic charge thereto. It comprises a support carrying a photoconductive insulating layer, which layer

comprises at least one photoconductive substance consisting of a 2,5-bis (para-aminophenyl)-1,3,4-oxadiazole compound. In preferred embodiments of the invention, the said photoconductive substance or at least one of the said photoconductive substances is of the general formula:



or



in which R<sub>1</sub> represents hydrogen or an alkyl, acyl, or cycloalkyl radical,

R<sub>2</sub> represents hydrogen,

R<sub>3</sub> represents an alkyl or acyl radical,

R<sub>4</sub> represents an alkyl radical,

and

R<sub>5</sub> represents hydrogen or alkyl.

Compounds of these general formulae include, for example,

30 2,5-bis-[4'-aminophenyl-(1')]-1,3,4-oxadiazole, the 2,5-bis-[4'-monoalkylamino-phenyl-(1')]-1,3,4-

oxadiazoles,

the 2,5-bis-[4'-dialkylamino-phenyl-(1')]-1,3,4-

oxadiazoles,

the 2,5-bis-[4'-monoacylaminophenyl-(1')]-1,3,4-

oxadiazoles,

to mention only a few of the most important.

40 The 2,5-bis-(p-amino-phenyl)-1,3,4-oxadiazole compounds can generally be prepared by methods known per se from 2 mols of the appropriate para-aminobenzene carboxylic acid and 1 mol of a hydrazine salt in the presence of dehydrating agents, such as oleum or polyphosphoric acid.

45 The 2,5-bis-(para-amino-phenyl)-1,3,4-oxadiazole compounds have very good photoconductivity and are particularly suitable for the preparation of homogeneous layers having a long shelf-life. The compounds are colourless and fluoresce in daylight or in ultraviolet light.

50 Compounds which are particularly adaptable to the present invention have the following formulae:

FORMULA 1



FORMULA 2



FORMULA 3



FORMULA 4





The photoconductive substances which are used according to the invention for the preparation of the photoconductive insulating layers are preferably so used in solution in organic solvents such as for example benzene, acetone,

methylene chloride or ethylene-glycol-monomethyl-ether. Mixtures of two or more photoconductive substances may be used, also in such solution. Mixtures of solvents may also be used. It is also possible to employ the photoconductive substances in association with other organic photoconductive substances.

It has further been found advantageous in preparing the photoconductive insulating layers to use the photoconductive substance or substances in association with a resin, synthetic polymer or other organic colloid, for example:

(a) natural and synthetic resins, e.g. balsam resins, phenol resins and other resins modified with colophony, coumarone resins and indene resins and the substances covered by the collective term "synthetic lacquer resins," 5 which includes processed natural substances such as cellulose ether, see the Kunststofftaschenbuch (Plastic Pocket Book) published by Saechtling-Zebrowski (11th edition, 1955, page 212 onwards);

(b) polymers (including co-polymers) such as the polyvinyl chlorides, polyvinyl acetate, polyvinyl acetals, polyvinyl alcohols, polyvinyl ethers, polyacrylic and polymethacrylic esters, and polystyrene and isobutylene polymers:

acrylic esters, and polystyrene and isobutylene polymers; (c) polycondensates, e.g., polyesters, such as phthalate resins, alkyd resins, maleic acid resins, colophony esters of mixed higher alcohols, phenol-formaldehyde resins, particularly colophony-modified phenol-formaldehyde condensates, urea-formaldehyde resins, melamine-formaldehyde condensates, aldehyde resins, ketone resins of which particular mention is to be made of AW 2 resins of the firm Badische Anilin- und Sodaefabrik, xylene-formaldehyde resins and polyamides; and

(d) polyadducts, such as polyurethanes.

When the photoconductive substances are employed in association with organic colloids, the proportion of resin to photoconductive substance can be varied very greatly. The use of mixtures of approximately equal parts by weight of resin or other colloid and photoconductive substance has been found generally advantageous. When such mixtures of approximately equal parts by weight of resin and photoconductive substance are used, in most cases said solutions give homogeneous transparent colourless layers on drying that can be considered as solid solutions.

The support may be of any material suitable for use in 5 electrophotographic processes, for example, aluminum or other metal plates or foils; glass plates; paper sheets or webs, or plastic foil, especially foils made of electrically conductive resins. If paper is to be used as support for the 0 photoconductive layer, it is preferable that it shall have been pretreated against penetration by the coating solution, for example with methyl-cellulose in aqueous solution; polyvinyl alcohol in aqueous solution; a solution in acetone and methyl-ethyl-ketone of a mixed polymer of 5 acrylic acid methyl ester and acrylonitrile; or with solutions of polyamides in aqueous alcohols. Aqueous dispersions of other substances suitable for the pretreatment 0 of the paper surface may also be used.

Solutions of the photoconductive substances in organic solvents as described above, with or without the added organic colloids aforementioned, can be applied to the supports in known manner (for example, by spraying, direct application, or whirl coating), and the supports thus coated, dried, so that an even photoconductive layer is formed thereon.

While the layers are, in themselves, non-light-sensitive, by applying a positive or negative electrostatic charge thereto, by means for example, of a corona discharge, the layers are rendered light-sensitive and can be used with long-wave U.V. light of 3600 to 4000 A.U. in producing electrostatic latent images as described above. Very good images may be obtained by a short exposure under a master to a high-pressure mercury vapour lamp.

Although the layers when charged are but slightly sensitive to light in the visible spectrum, it has further been

found that their spectral sensitivity can be extended into the visible part of the spectrum by the addition to the layers of sensitizers, preferably in the proportion one to three percent weight for weight of photoconductive substance. The most suitable sensitizers are dyestuff compounds, a number of which are given by way of example in the following table:

| Dyestuff Group      | Dyestuff compound                                                                                                | Reference<br>(Schultz' Farbstofftabellen, 7th edn.,<br>vol. 1 (1931))                                                                                                |
|---------------------|------------------------------------------------------------------------------------------------------------------|----------------------------------------------------------------------------------------------------------------------------------------------------------------------|
| Triarylmethane dyes | Brilliant Green<br>Victoria Blue B<br>Methyl Violet<br>Crystal Violet<br>Acid Violet 6B                          | No. 760 (p. 314).<br>No. 822 (p. 347).<br>No. 783 (p. 327).<br>No. 785 (p. 329).<br>No. 831 (p. 351).                                                                |
| Xanthene dyes:      |                                                                                                                  |                                                                                                                                                                      |
| Rhodamines          | Rhodamine B<br>Rhodamine 6G<br>Rhodamine G extra<br>Sulphorhodamine B<br>True acid Eosin G<br>Eosin S<br>Eosin A | No. 864 (p. 365).<br>No. 866 (p. 366).<br>No. 865 (p. 366).<br>No. 863 (p. 364).<br>No. 870 (p. 369).<br>No. 883 (p. 375).<br>No. 881 (p. 374).<br>No. 886 (p. 376). |
| Pthaleins           | Erythrosin<br>Phloxin<br>Rose Bengal<br>Fluorescein                                                              | No. 890 (p. 378).<br>No. 889 (p. 378).<br>No. 880 (p. 373).<br>No. 1038 (p. 449).                                                                                    |
| Thiazine dyes       | Methylene blue                                                                                                   | No. 901 (p. 383).                                                                                                                                                    |
| Acridine dyes       | Acridine yellow<br>Acridine orange                                                                               | No. 908 (p. 387).<br>No. 906 (p. 386).                                                                                                                               |
| Quinoline dyes      | Tryptavine<br>Pinacyanol<br>Cryptocyanine                                                                        | No. 924 (p. 396).<br>No. 927 (p. 397).                                                                                                                               |
| Quinone dyestuffs   |                                                                                                                  |                                                                                                                                                                      |
| Anthraquinones      | Alizarin<br>Alizarin red S<br>Quinizarine                                                                        | No. 1141 (p. 499).<br>No. 1145 (p. 502).<br>No. 1148 (p. 504).                                                                                                       |
| Cyanine dyes        |                                                                                                                  |                                                                                                                                                                      |

The layer-carrying supports may be utilized for the production of images by electrophotographic means, for example, as follows: When the photoconductive layer has been charged, by means of, for example, a corona discharge with a charging apparatus maintained at 6000 volts, the thus sensitized layer is exposed to light under a master or by episcopic or diascopic projection and is then dusted over in known manner with a suitable developing agent such as a resin powder coloured with carbon black. We prefer a resin developer obtained by fusing 30 parts by weight of polystyrene (K-Wert 55), 30 parts by weight of a maleic acid resin modified with rosin and sold under the registered trade-mark "Beckacite K 105," and 3 parts by weight of carbon black, and subsequently finely grinding the fused mass. The image that now becomes visible can easily be wiped off, and therefore needs to be fixed; it can, for example, be heated briefly to approximately 120° C. by means of an infra-red radiator. The temperature need not be as high as this if the heat treatment is carried out in the presence of vapours of solvents such as trichloroethylene, carbon tetrachloride or ethyl alcohol. The powdered image can also be fixed by means of steam. From positive masters, positive images of good contrast are produced.

After being fixed these electrophotographic images can be converted into printing plates; the support, e.g., the paper or plastic foil, is wiped over with a solvent for the photoconductive layer, e.g., alcohol, or acetic acid, and then rinsed with water and rubbed in with greasy ink in known manner. In this way positive printing plates are obtained which can be set up in an offset machine and used for printing. They give very long runs.

If transparent supports are used the electrophotographic images can also be used as masters for the production of further copies on any sort of light-sensitive sheets. In this respect the photoconductive compounds to be used

as provided by the invention are superior to substances used hitherto, such as selenium or zinc oxide, inasmuch as the latter give cloudy layers because solid solutions cannot be produced with such materials and only suspensions are possible.

Where translucent supports are used for photoconductive layers such as are provided by this invention, reflex images can also be produced. The possibility of a reflex copy is also an advantage over the known art.

Moreover the photoconductive layers prepared as provided in the invention have a further important advantage in that they can be charged positively as well as negatively. With positive charging the images are particularly good while there is negligible evolution of ozone, which is considerable with negative charging.

The invention and methods of practicing the same are further illustrated in the following specific examples, in which reference is made to the chemical formulae listed above:

#### Example 1

A solution containing 1 g. of 2,5-bis-[4'-dimethylamino-phenyl-(1')]-1,3,4-oxadiazole, corresponding to Formula 1, and 1 g. of indene resin (e.g., the product obtainable from Farbenfabriken Bayer AG, Leverkusen, under the trade named "TC-Harz") dissolved in 30 g. of benzene, is applied to a paper foil the surface of which has been pretreated to prevent the penetration of organic solvents. The treated paper is then dried.

On this treated paper, direct images are produced by the electrophotographic process whereby, by means of a corona discharge apparatus, the paper is given either a positive or a negative electric charge; it is then exposed under a positive master to a high-pressure mercury lamp and dusted with a resin powder coloured with carbon black. The finely powdered resin adheres to those parts of the layer that were not exposed to light during exposure and a positive image is developed: this is heated slightly and thereby stabilised (fixed). It shows good contrast since the background of the paper is brightened by the substances that have been applied thereto.

If instead of paper as above, a suitable transparent plastic foil or transparent paper is used as support for the photoelectric layer, the images produced are suitable as master-copies for duplication processes by means of any sort of light-sensitive sheets.

The compound corresponding to Formula 1 may be produced as follows: 36 g. of 4-dimethylamino-benzoic acid are introduced, with cooling, into a solution of 13 g. of hydrazine sulphate in 250 g. of oleum (24% SO<sub>3</sub>). The reaction mixture is then heated with agitation to 60-70° C. for 2-3 hours; it is then poured onto ice and, with cooling, made slightly alkaline by means of sodium hydroxide solution; the precipitated condensation product is separated from the mother liquor. The oxadiazole compound formed (Formula 1) is washed and dried; it is in the form of a light powder, which in solution gives bluish fluorescence in ultra-violet light. The compound has a melting point of 225-227° C.

#### Example 2

A solution containing 1 g. of 2,5-bis-[4'-diethylamino-phenyl-(1')]-1,3,4-oxadiazole corresponding to Formula 2 and 2 g. of coumarone resin (for example the type known as 701/70 from the Gesellschaft für Teerverwertung, Duisburg-Meiderich) in 30 g. of methylene chloride, is applied to an aluminum foil. After the solvent has evaporated, the oxadiazole layer adheres firmly to the aluminum surface. With this coated aluminum foil, electrophotographic images can be produced as described in Example 1. If a sheet of paper is laid upon the unfixed image in carbon black-resin powder, and recharging by means of a corona discharge is carried out, the carbon black-resin image is transferred to transparent paper or transparent plastic foil, the image obtained can be further copied, for example on diazo photoprinting paper.

The compound corresponding to Formula 2, can be prepared from 13 g. of hydrazine sulfate and 42 g. of 4-diethylaminobenzoic acid in 260 g. of oleum (24% SO<sub>3</sub>), in analogous manner to the compound corresponding to Formula 1. The reaction mixture is heated with agitation for three hours to 60-70° C.; it is then poured on to ice and, with cooling, made slightly alkaline with sodium hydroxide; the precipitated condensation product is separated from the mother liquor. It is purified by recrystallization from 96% ethyl alcohol and melts at 152-153° C.

Instead of oleum, polyphosphoric acid can be employed as condensation agent in the above-described process. In such case 13 g. of hydrazine sulphate are introduced into 200 g. of polyphosphoric acid at room temperature and then 42 g. of 4-diethylamino-benzoic acid are added and the mixture is heated for two hours to 80° C. When everything has gone into solution the syruplike condensation product is poured on to ice. The precipitate is separated from the mother liquor, rinsed in water and recrystallized from 96% alcohol.

#### Example 3

1.5 g. of the compound corresponding to Formula 1, 0.5 g. of the compound corresponding to Formula 2, and 1 g. of a synthetic resin produced by condensation of cyclohexanone with methylcyclohexanone (e.g. the product of Badische Anilin und Soda-Fabrik, Ludwigshafen, known as Kunstharsz AW2) are dissolved in 50 g. of benzene and then applied to paper which has been prepared in accordance with U.S. Patents Nos. 2,534,650, 2,681,617, or 2,559,610. The layer left on the paper after evaporation of the solvent adheres firmly to the surface. With coated paper of this kind, images with good contrast on white ground are produced by the electrophotographic process as described in Example 1. If it is desired to produce a printing plate, the image is fixed by heating and the image side of paper wiped over with 96% ethyl alcohol or 50% acetic acid, rinsed with water and rubbed in with greasy ink and 1% phosphoric acid. From positive masters positive printing plates are obtained from which printing can be carried out by means of an offset machine.

#### Example 4

0.5 g. of 2,5-bis-[4'-isoamylamino-phenyl-(1')]-1,3,4-oxadiazole corresponding to Formula 3, 1.5 g. of 2,5-bis-[4'-n-propylamino-phenyl-(1')]-1,3,4-oxadiazole corresponding to Formula 4, 1 g. of colophony-formaldehyde resin (e.g., that marketed by Farbenfabriken Bayer AG, Leverkusen, under the registered trade-mark "Corepal 140") and 0.01 g. of methylene blue are dissolved in 30 g. of benzene and the solution is applied to a paper foil of the kind employed in Example 1 and dried. The paper coated in this manner is electrically charged in known manner and can be discharged by exposure to a high-pressure mercury vapour or to an incandescent lamp, whereby, if a master is interposed, an image of the master copy is produced. The addition of the methylene blue as sensitizer enables the exposure time to be reduced to a fifth of that required in the absence of the sensitizer.

The compound corresponding to Formula 3 may be obtained by the introduction with cooling of 43 g. of 4-isoamylamino-benzoic acid into a solution of 13 g. of hydrazine sulfate in 250 g. of oleum (24% SO<sub>3</sub>) followed by further treatment of the reaction mixture in analogous manner to that given in Example 1 for the compound with Formula 1; the compound corresponding to Formula 3 melts at 130-132° C. The compound corresponding to Formula 4 may be prepared in analogous manner, 39 g. of 4-n-propylamino-benzoic acid being used; it melts at 137-139° C. Polyphosphoric acid can be used instead of oleum in the preparation of both compounds.

#### Example 5

A paper foil is coated with a solution, and the other

procedures followed, as in Example 4, except that in the solution, one or both of the compounds corresponding to Formulae 3 and 4 are replaced by the same respective quantities of the compound 2,5-bis-[4'-cyclopentylamino-phenyl-(1')]-1,3,4-oxadiazole corresponding to Formula 5. This compound, which melts at 118-120° C., can be prepared by condensing 13 g. of hydrazine sulfate with 41 g. of 4-cyclopentylamino-benzoic acid in 250 g. of oleum in a manner analogous to that given in Example 1 for the preparation of the compound of Formula 1. The compound 4-cyclopentylamino-benzoic acid is obtained when 68.5 g. of 4-amino-benzoic acid are dissolved with 33 g. of potassium carbonate in 300 cc. of water and the solution is boiled for six hours under reflux with 74.5 g. of cyclopentyl bromide. After the reaction mixture has cooled, crystals are precipitated which are recrystallized from 96% ethyl alcohol. The 4-cyclopentylamino-benzoic acid melts at 128-130° C.

20

#### Example 6

0.5 g. of 2,5-bis-[4'-cyclohexylamino-phenyl-(1')]-1,3,4-oxadiazole (Formula 6); 1 g. of 2,5-bis-[4'-n-propylamino-phenyl-(1')]-1,3,4-oxadiazole (Formula 7) and 1 g. of resin-modified maleic acid resin (e.g., that marketed by Reichhold Chemie AG, Hamburg, under the registered trade-mark "Beckacite K 125") are dissolved in 30 g. of benzene and the benzene solution is applied to a superficially-roughened aluminum foil. After the solvent has evaporated, the layer left behind adheres firmly to the surface of the foil. For the production of an image, subsequent procedure is the same as described in Example 1, a positive image being obtained from a positive master; fixing is also carried out as described in Example 1. To convert the image into a positive printing plate, the image side of the aluminum foil is wiped over with ethyl alcohol (96%), rinsed with water and rubbed in with greasy ink and 1% phosphoric acid.

40 2,5-bis-[4'-cyclohexylamino-phenyl-(1')]-1,3,4-oxadiazole (Melting Point: 186-187° C.) can be obtained by condensation of 13 g. of hydrazine sulfate with 48 g. of 4-cyclohexylamino-benzoic acid in 260 g. of oleum (24% SO<sub>3</sub>) in analogous manner to the compound corresponding to Formula 1, which is described in Example 1. 2,5-bis-[4'-n-propylamino-phenyl-(1')]-1,3,4-oxadiazole (Melting Point: 137-138° C.) can be obtained from 13 g. of hydrazine sulfate and 48 g. of 4-di-n-propyl-amino-benzoic acid in oleum, also in analogous manner to that in Example 1.

#### Example 7

0.5 g. each of 2,5-bis-[4'-acetylamino-phenyl-(1')]-1,3,4-oxadiazole (Formula 8) and 2,5-bis-[4'-acetyl-amino-2'-chlorophenyl-(1')]-1,3,4-oxadiazole (Formula 9) together with 1 g. of resin-modified maleic acid resin (e.g., that marketed by Reichhold Chemie AG, Hamburg, under the registered trade-mark "Beckacite K 105") are dissolved in 30 g. of methylene chloride and the solution is coated on to a paper foil of the same type as used in Example 1, and dried. The paper foil is then further processed for the production of an image as described in Example 1. A positive image is obtained from a positive master.

65 In analogous manner to that described in Example 1 for the preparation of the compound of Formula 1, 2,5-bis-[4'-acetylamino-phenyl-(1')]-1,3,4-oxadiazole (Melting Point: 262-263° C.) can be obtained by condensation of 13 g. of hydrazine sulfate with 39 g. of 4-acetyl-amino-benzoic acid in 250 g. of oleum (24% SO<sub>3</sub>); and 2,5-bis-[4'-acetylamino-2-(chlorophenyl)-(1')]-1,3,4-oxadiazole (Melting Point: 169-170° C.) can be obtained by condensation of 13 g. of hydrazine sulfate with 21 g. of 4-acetylamino-2-chloro-benzoic acid in 240 g. of oleum (24% SO<sub>3</sub>).

## 9

## Example 8

The procedures of Example 7 are followed, except that in the coating solution, one or both of the compounds corresponding to Formulae 8 and 9 or are replaced by the same quantities of 2,5-bis-[4'-(n-propylamino)-2'-chlorophenyl-(1')]-1,3,4-oxadiazole (Formula 10).

In analogous manner to that described in Example 1 for preparing the compound of Formula 1, 2,5-bis-[4'-(n-propylamino)-2'-chlorophenyl-(1')]-1,3,4-oxadiazole (Melting Point: 132-140° C.) can be prepared by condensation of 13 g. of hydrazine sulfate with 45 g. of 4-n-propylamino-2-chloro-benzoic acid in 260 g. of oleum (24% SO<sub>3</sub>).

## Example 9

1 g. of 2,5-bis-[4'-diethylamino-phenyl-(1')]-1,3,4-oxadiazole (Formula 2) and 1 g. of phenol-modified synthetic resin (e.g. the resin produced by polycondensation and marketed under the registered trade-mark "Rhenophen 140" by Rheinpreussen G.m.b.H. Homberg-am-Niederrhein) are dissolved in 30 g. of benzene. This solution is coated on to a translucent paper (i.e. paper which is light-permeable but not transparent), the surface of which paper has been pretreated against penetration of organic solvents, and the coated paper is dried.

The treated paper is electrically charged by means of a corona discharge and placed with its coated side against a page of a book which is printed on both sides and against the back of which page a sheet of black paper has been placed, and it is exposed for four seconds to the light of a 100-watt incandescent lamp, i.e., exposure takes place through the translucent paper. After the exposure, the reflex image is dusted over with a resin powder coloured with carbon black. A positive mirror-image with good contrast is obtained. If paper or plastic foil is firmly pressed upon the image so obtained, the image is transferred and a correct reading image is produced on the paper or foil. In the production of the correct reading image an electric field can be applied in manner known per se to the paper or foil which is to receive the correct reading image. If the paper or foil is transparent, intermediate originals are obtained suitable for further reproduction, for example on photo-printing paper.

## Example 10

1 g. of 2,5-bis-[4'-ethylamino-phenyl-(1')]-1,3,4-oxadiazole corresponding to Formula 11 and 1 g. of ketone resin (for example that known as Kunsthärz EM marketed by Rheinpreussen G.m.b.H., Homberg-am-Niederrhein) are dissolved in 30 g. of ethylene glycol-monomethyl-ether and the solution is coated on to paper and dried. For the production of an image, the coated paper foil is further processed as described in Example 1. From a positive master a positive image with good contrast is obtained.

2,5-bis-[4'-ethylamino-phenyl-(1')]-1,3,4-oxadiazole (Formula 11), with Melting Point 160-161° C. can be obtained by condensation of 36 g. of 4-mono-N-ethylamino-1-benzoic acid with 13 g. of hydrazine sulfate in 250 g. of oleum (24% SO<sub>3</sub>) in analogous manner to that described in Example 1 for the preparation of the compound of Formula 1.

## Example 11

1 g. of the compound corresponding to Formula 12, 1 g. of ketone resin (e.g., the Kunsthärz EM mentioned in Example 8) and 0.01 g. of rhodamine B (see the preceding table of dyestuffs) are dissolved in 30 g. of glycolethylene-monomethylether and the solution is coated on to paper and dried.

The sheet is charged by means of a corona discharge, and the thus sensitized paper is exposed for 1/2 second under a positive master to the light of a 100-watt incandescent lamp and then dusted over with resin powder coloured with carbon black. A positive image is pro-

## 10

duced which is fixed by heating. Black images on a colourless ground are obtained.

The compound corresponding to Formula 12, 2,5-bis-[4' - N - ethyl - N - n - propyl - aminophenyl - (1')]-1,3,4-oxadiazole with Melting Point 98° C. can be prepared by condensation of 20.5 g. of 4-N-ethyl-N-n-propyl-amino-benzoic acid with 13 g. of hydrazine sulfate in 250 g. of oleum (24% SO<sub>3</sub>) in analogous manner to that given in Example 1 for the compound corresponding to Formula 1.

The N-ethyl-N-n-propyl-amino-benzoic acid can be obtained in manner analogous to that described in Example 5 for the preparation of 4-cyclopentyl-amino-benzoic acid, a solution of 16.5 g. of 4-N-ethyl-amino-benzoic acid and 13.8 g. of potassium carbonate in 80 cc. of water to which 12.3 g. of propyl bromide has been added being boiled under reflux for a number of hours.

## Example 12

20 The procedure as in Example 1, is followed, except that a solution of 0.5 g. of the compound corresponding to Formula 2 and 0.5 g. of the compound corresponding to Formula 11 in 30 g. of ethylene-glycol-monomethyl-ether is used. The images obtained are of good contrast and positives are obtained from positive masters. Reproductions can also be made from pages printed on both sides by episcopic projection. Half and whole tones are reproduced with good contrast.

## 30

## Example 13

1 g. of the compound corresponding to Formula 13, 1 g. of ketone resin (e.g., the Kunsthärz EM mentioned in Example 8) and 0.02 g. of the cyanine dyestuff of the following structure:



are dissolved in 30 g. of ethylene-glycol-monomethyl-ether and the solution is coated on to paper and dried.

The sheet is charged by means of a corona discharge, 45 and is then exposed for one second under a positive master to the light of a 100-watt incandescent lamp at a distance of about 15 cm. and then dusted over with a resin powder coloured with carbon black as described in Example 1. A positive image is formed which is fixed by heating.

The compound corresponding to Formula 13, 2,5-bis-[4' - (N - ethyl - N - acetyl) - amino - phenyl - (1')]-1,3,4-oxadiazole of Melting Point 156-157° C. can be prepared from the compound of Formula 11, by boiling the same for four hours with acetic anhydride. When the reaction is complete, the resultant mass is poured on to water and after several hours the compound corresponding to Formula 13 precipitates out and after being rinsed with water is recrystallized from ethyl alcohol.

## 60

## Example 14

1 g. of the compound corresponding to Formula 1, 1 g. of a zinc resinate (for example that known as Zink-resinate 357, produced by Lehmann & Crebert, Mannheim-Rheinau) and 0.02 g. of acid violet 7 BN (see preceding table of dyestuffs) are dissolved in 30 g. of ethylene glycol-monomethyl-ether and coated on to paper and dried. After the material has been charged by means of a corona

70 discharge the sensitized paper is exposed under a positive master for 1/4 second at a distance of approximately 15 cm. to the light of a 100-watt incandescent lamp and then dusted over with a resin powder coloured with carbon black as described in Example 1. A positive image is formed that is fixed by heating.

## 75

*Example 15*

The procedure described in Example 1 is followed, except that a solution of 1 g. of the compound corresponding to Formula 11 and 1.5 g. of a polymerized natural resin (e.g., the resin produced by the American firm Hercules Powder Company, Wilmington, and marketed under the name Hercules "Poly Pale") in 30 g. of ethylene glycolmonomethyl-ether is used for coating paper. Positive images are obtained.

Instead of the above-mentioned resin produced by Hercules Powder Company, a resin consisting chiefly of dimerised abietinic acid can be used (e.g., Hercules "Dymerex" produced by the same firm) or a hydrogenated natural resin (e.g., Hercules "Staybelite" also produced by Hercules Powder Company).

*Example 16*

A paper base is coated with a solution of 10 g. of after-chlorinated polyvinyl chloride (e.g., the plastic marketed by Dynamit AG, Rheinfelden, under the trade name "Rhenoflex") in 100 g. of acetone, and dried. After drying, this paper is coated with a solution of 1 g. of the compound corresponding to Formula 2 and 1 g. of ketone resin (e.g., that known as Kunstharsz AP produced by Chemische Werke Hüls AG, Marl) in 30 g. of ethyleneglycol-monomethyl-ether and further processed as described in Example 1.

The paper is given a positive charge to sensitize the same, and is then exposed beneath a master at a distance of approximately 15 cm. to the light of a 100-watt incandescent lamp; images with good contrast are obtained after an exposure of only one second.

*Example 17*

1 g. of 2-[4'-diethylamino-phenyl-(1')]-5-[4"-dimethylamino-phenyl-(1')]-1,3,4-oxadiazole corresponding to Formula 14 and 1 g. of manila copal or other natural resin, are dissolved in 50 g. of ethyleneglycol-monomethyl-ether. The solution is applied to transparent paper and dried. Further procedure is as described in Example 1. The electrophotographically produced images are suitable as masters for the preparation of reproductions on any light-sensitive surfaces.

Instead of the compound corresponding to Formula 14, 2-[4'-dimethylamino-phenyl-(1')]-5-[4"-amino-3"-chloro-phenyl-(1')]-1,3,4-oxadiazole, corresponding to Formula 17, may be used.

The compound corresponding to Formula 14 can be prepared as follows: Into a solution of 13 g. of hydrazine sulphate in 250 g. of oleum (24% SO<sub>3</sub>) a mixture is introduced consisting of 19.3 g. of 4-diethylamino-benzoic acid and 16.5 g. of 4-dimethylamino-benzoic acid, the temperature being maintained by cooling at approximately 25° C. The reaction mixture is then heated with stirring for four hours at 60° C. The reaction mixture is then poured upon ice and made slightly alkaline by the addition with cooling upon ice and made slightly alkaline by the addition with cooling of sodium hydroxide solution; the condensation product which then precipitates out is separated by suction, washed with water and purified by recrystallization from 80% ethyl alcohol. 2,5-bis-[4"-dimethyl-amino-phenyl(1')]-1,3,4-oxadiazole (Formula 1) which is sparingly soluble is formed as a by-product and is separated by repeated recrystallization of the reaction product from 80% ethyl alcohol. 2-[4'-diethylamino-phenyl-(1')]-5-[4"-dimethylamino-phenyl-(1')]-1,3,4-oxadiazole melts, after recrystallization, at 158-160° C.

The compound corresponding to Formula 17 is obtained, in analogous manner to the compound corresponding to Formula 14, from 13 g. of hydrazine sulfate, 250 g. of oleum (24% SO<sub>3</sub>) and a mixture of 16.5 g. of 4-dimethyl-amino-benzoic acid and 17.2 g. of 4-amino-3-chloro-benzoic acid. The compound corresponding to For-

mula 17, 2-[4'-dimethylamino-phenyl-(1')]-5-[4"-amino-3"-chloro-phenyl-(1")]-1,3,4-oxadiazole, is obtained by repeated recrystallization of the reaction product from 80% ethyl alcohol. It melts at 216-217° C.

*Example 18*

The procedure as in Example 1, is followed except that the paper-foil is coated with a solution of 1 g. of 2-[4'-mono-n-propylamino-phenyl-(1')]-5-[4"-dimethylamino-phenyl-(1")]-1,3,4-oxadiazole corresponding to Formula 15 and 1 g. of 2-[4'-mono-n-propylamino-phenyl-(1')]-5-[4"-monoethylamino-phenyl-(1")]-1,3,4-oxadiazole corresponding to Formula 16 in 30 g. of glycol-monomethyl-ether. Images electrophotographically produced therewith have very good contrast.

The compound corresponding to Formula 15 can be produced, in analogous manner to the compound corresponding to Formula 14, from 13 g. of hydrazine sulfate dissolved in 250 g. of oleum (24% SO<sub>3</sub>) and a mixture of 17.9 g. of 4-mono-n-propylamino-benzoic acid and 16.5 g. of 4-dimethylamino-benzoic acid. The reaction product, 2-[4'-mono-n-propylamino-phenyl-(1')]-5-[4"-dimethylamino-phenyl-(1")]-1,3,4-oxadiazole is purified by fractional recrystallization from 80% ethyl alcohol and has a Melting Point of 148-150° C.

The compound corresponding to Formula 16 can also be produced in analogous manner to the compound corresponding to Formula 14.

After 13 g. of hydrazine sulfate have been dissolved in 250 g. of oleum (24% SO<sub>3</sub>), a mixture of 17.9 g. of 4-mono-n-propylamino-benzoic acid and 16.5 g. of 4-monoethylamino-benzoic acid is introduced into the solution. Treatment of the reaction mixture is as in the preparation described of the compound corresponding to Formula 14. The reaction product, 2-[4'-mono-n-propylamino-phenyl-(1')]-5-[4"-monoethyl-amino-phenyl(1")]-1,3,4-oxadiazole, is purified by recrystallization from 80% ethyl alcohol; it melts at 126-127° C.

*Example 19*

10 g. of after-chlorinated polyvinylchloride, e.g., a product traded under the registered trademark "Rhenoflex" by Dynamit-Aktion-Gesellschaft (formerly Alfred Nobel & Co.) of Troisdorf, Rheinfelden, plants, are dissolved in 100 g. of methyl ethyl ketone. To this solution there are added first 10 g. of the compound corresponding to Formula 1, dissolved in 50 g. of toluene, and then 0.011 g. of Rhodamine B extra (see Schultz, "Farbstofftabellen," 7th edition, vol. 1, 1931, No. 864, page 365), dissolved in 2 g. of methanol. This mixed solution, which has a kinetic viscosity of about 20.8 centistokes (17.1 centipoises) is used for coating paper by means of a casting equipment in such a way that a layer of about 6 microns in thickness is obtained. As described in Example 1, direct images are produced on this paper by an electrophotographic process. The degree of light-sensitivity of the paper is very high. By way of an episcopic process and using a light source of about 30 lux, good contrast images may be produced with an exposure of 1 second from originals printed on both sides.

*Example 20*

10 g. of a product obtained by subsequent chlorination of polyvinylchloride, e.g., of the product sold under the registered trade-mark "Rhenoflex" by Dynamit-Aktiengesellschaft, Rheinfelden, are dissolved in 100 g. of methyl-ethyl-ketone. To this solution there is added first a solution containing 10 g. of the compound corresponding to Formula 1 in 50 g. of toluene, then a solution containing 0.004 g. of ethyl violet (see "Farbstofftabellen," 7th edition, volume 1 (1931), No. 787, page 331), in 2 g. of methanol. The solution thus obtained, which has a kinetic viscosity of about 20.8 centistokes (17.1 centipoises), is used for mechanically coating a paper base. Advantageously the coat should have a thickness of about 6

microns. After drying the coated layer the paper is given a negative charge by means of a corona discharge, and then a latent image of a book page, printed on both sides is produced on the layer by an episcopic process. The layer side of the paper is then treated with a developer consisting of very small glass balls coloured by means of a very finely divided resin-carbon black mixture. The black resin adheres to those areas of the layer which during exposure were not struck by light, and a positive image becomes visible which is fixed by slight heating. The image has good contrast.

What is claimed is:

1. An electrophotographic material comprising an electrically conductive support layer and a photoconductive insulating layer, the latter containing a 2,5-bis-(p-aminophenyl)-1,3,4-oxadiazole and a dyestuff sensitizer.

2. An electrophotographic material comprising an electrically conductive support layer and a photoconductive insulating layer, the latter containing a dyestuff sensitizer and a compound having the formula



in which R, R<sub>1</sub>, R<sub>2</sub> and R<sub>3</sub> are selected from the group consisting of hydrogen, alkyl, cycloalkyl, and acyl radicals; and X and X<sub>1</sub> are selected from the group consisting of hydrogen and halogen.

3. An electrophotographic material comprising an electrically conductive support layer and a photoconductive insulating layer, the latter containing a dyestuff sensitizer and a compound having the formula



in which R, R<sub>1</sub>, R<sub>2</sub>, and R<sub>3</sub> are alkyl radicals and X and X<sub>1</sub> are selected from the group consisting of hydrogen and halogen.

4. An electrophotographic material comprising an electrically conductive support layer and a photoconductive insulating layer, the latter containing a dyestuff sensitizer and a compound having the formula



in which R and R<sub>2</sub> are hydrogen and R<sub>1</sub>, and R<sub>3</sub> are alkyl radicals.

5. An electrophotographic material comprising an electrically conductive support layer and a photoconductive insulating layer, the latter containing a dyestuff sensitizer and a compound having the formula



in which R and R<sub>2</sub> are hydrogen and R<sub>1</sub> and R<sub>3</sub> are acyl radicals.

6. A photographic reproduction process which comprises exposing an electrically charged, supported photoconductive insulating layer to light under a master and developing the resulting image, the photoconductive layer comprising a 2,5-bis-(p-aminophenyl)-1,3,4-oxadiazole.

7. A process according to claim 6 in which the photoconductive layer contains a dyestuff sensitizer.

8. A process according to claim 6 in which the photoconductive layer contains an organic colloid.

9. A photographic reproduction process which comprises exposing an electrically charged, supported photoconductive insulating layer to light under a master and

developing the resulting image, the photoconductive layer comprising a compound having the formula



in which R, R<sub>1</sub>, R<sub>2</sub>, and R<sub>3</sub> are selected from the group consisting of hydrogen, alkyl, cycloalkyl, and acyl radicals; and X and X<sub>1</sub> are selected from the group consisting of hydrogen and halogen.

10. A process according to claim 9 in which the photoconductive layer contains a dyestuff sensitizer.

11. A process according to claim 9 in which the photoconductive layer contains an organic colloid.

12. A photographic reproduction process which comprises exposing an electrically charged, supported photoconductive insulating layer to light under a master and developing the resulting image, the photoconductive layer comprising a compound having the formula



in which R, R<sub>1</sub>, R<sub>2</sub>, and R<sub>3</sub> are alkyl radicals and X and X<sub>1</sub> are selected from the group consisting of hydrogen and halogen.

13. A process according to claim 12 in which the photoconductive layer contains a dyestuff sensitizer.

14. A process according to claim 12 in which the photoconductive layer contains an organic colloid.

15. A photographic reproduction process which comprises exposing an electrically charged, supported photoconductive insulating layer to light under a master and developing the resulting image, the photoconductive layer comprising a compound having the formula



in which R and R<sub>2</sub> are hydrogen and R<sub>1</sub> and R<sub>3</sub> are alkyl radicals.

16. A process according to claim 15 in which the photoconductive layer contains a dyestuff sensitizer.

17. A process according to claim 15 in which the photoconductive layer contains an organic colloid.

18. A photographic reproduction process which comprises exposing an electrically charged, supported photoconductive insulating layer to light under a master and developing the resulting image, the photoconductive layer comprising a compound having the formula



in which R and R<sub>2</sub> are hydrogen and R<sub>1</sub> and R<sub>3</sub> are acyl radicals.

19. A process according to claim 18 in which the photoconductive layer contains a dyestuff sensitizer.

20. A process according to claim 18 in which the photoconductive layer contains an organic colloid.

21. A photographic reproduction process which comprises exposing an electrically charged, supported photoconductive insulating layer to light under a master and developing the resulting image, the photoconductive layer comprising 2,5-bis-(4'-dimethylaminophenyl-(1'))-1,3,4-oxadiazole.

22. A photographic reproduction process which comprises exposing an electrically charged, supported photoconductive insulating layer to light under a master and

developing the resulting image, the photoconductive layer

comprising 2,5-bis-(4'-diethylaminophenyl-(1'))-1,3,4-oxadiazole.

23. A photographic reproduction process which comprises exposing an electrically charged, supported photoconductive insulating layer to light under a master and developing the resulting image, the photoconductive layer comprising 2,5-bis-(4'-isoamylaminophenyl-(1'))-1,3,4-oxadiazole.

24. A photographic reproduction process which comprises exposing an electrically charged, supported photoconductive insulating layer to light under a master and developing the resulting image, the photoconductive layer comprising 2,5-bis-(4'-cyclopentylaminophenyl-(1'))-1,3,4-oxadiazole.

25. A photographic reproduction process which comprises exposing an electrically charged, supported photoconductive insulating layer to light under a master and developing the resulting image, the photoconductive layer comprising 2,5-bis-(4'-cyclohexylaminophenyl-(1'))-1,3,4-oxadiazole.

26. A photographic reproduction process which comprises exposing an electrically charged, supported photoconductive insulating layer to light under a master and developing the resulting image, the photoconductive layer comprising 2,5-bis-(4'-di-n-propyl)-aminophenyl-(1'))-1,3,4-oxadiazole.

27. A photographic reproduction process which comprises exposing an electrically charged, supported photoconductive insulating layer to light under a master and developing the resulting image, the photoconductive layer comprising 2,5-bis-(4'-acetylaminophenyl-(1'))-1,3,4-oxadiazole.

28. A photographic reproduction process which comprises exposing an electrically charged, supported photoconductive insulating layer to light under a master and developing the resulting image, the photoconductive layer comprising 2,5-bis-(4'-acetylamo-2'-chlorophenyl-(1'))-1,3,4-oxadiazole.

29. A photographic reproduction process which comprises exposing an electrically charged, supported photoconductive insulating layer to light under a master and developing the resulting image, the photoconductive layer comprising 2,5-bis-(4'-n-proplamino)-2'-chlorophenyl-(1'))-1,3,4-oxadiazole.

30. A photographic reproduction process which comprises exposing an electrically charged, supported photoconductive insulating layer to light under a master and developing the resulting image, the photoconductive layer comprising 2,5-bis-(4'-ethylaminophenyl-(1'))-1,3,4-oxadiazole.

31. A photographic reproduction process which comprises exposing an electrically charged, supported photoconductive insulating layer to light under a master and developing the resulting image, the photoconductive layer comprising 2,5-bis-(4'-N-ethyl-N-n-propylaminophenyl-(1'))-1,3,4-oxadiazole.

32. A photographic reproduction process which comprises exposing an electrically charged, supported photoconductive insulating layer to light under a master and developing the resulting image, the photoconductive layer comprising 2,5-bis-(4'-N-ethyl-N-acetyl)-aminophenyl-(1'))-1,3,4-oxadiazole.

33. A photographic reproduction process which comprises exposing an electrically charged, supported photoconductive insulating layer to light under a master and developing the resulting image, the photoconductive layer comprising 2-(4'-diethylaminophenyl-(1'))-5-(4'-dimethylaminophenyl-(1'))-1,3,4-oxadiazole.

34. A photographic reproduction process which comprises exposing an electrically charged, supported photoconductive insulating layer to light under a master and developing the resulting image, the photoconductive layer comprising 2-(4'-dimethylaminophenyl-(1'))-5-(4'-amino-3'-chlorophenyl-(1'))-1,3,4-oxadiazole.

35. A photographic reproduction process which com-

prises exposing an electrically charged, supported photoconductive insulating layer to light under a master and developing the resulting image, the photoconductive layer comprising 2-(4'-mono-n-propylaminophenyl-(1'))-5-(4'-dimethylaminophenyl-(1'))-1,3,4-oxadiazole.

36. A photographic reproduction process which comprises exposing an electrically charged, supported photoconductive insulating layer to light under a master and developing the resulting image, the photoconductive layer comprising 2-(4'-mono-n-propylaminophenyl-(1'))-5-(4'-monoethylaminophenyl-(1'))-1,3,4-oxadiazole.

37. An electrophotographic material comprising an electrically conductive support layer and a photoconductive insulating layer, the latter containing a 2,5-bis-(p-aminophenyl)-1,3,4-oxadiazole and an organic colloid.

38. An electrophotographic material comprising an electrically conductive support layer and a photoconductive insulating layer, the latter containing an organic colloid and a compound having the formula



25 in which R, R<sub>1</sub>, R<sub>2</sub>, and R<sub>3</sub> are selected from the group consisting of hydrogen, alkyl, cycloalkyl, and acyl radicals; and X and X<sub>1</sub> are selected from the group consisting of hydrogen and halogen.

39. An electrophotographic material comprising an electrically conductive support layer and a photoconductive insulating layer, the latter containing an organic colloid and a compound having the formula



40 in which R, R<sub>1</sub>, R<sub>2</sub>, and R<sub>3</sub> are alkyl radicals and X and X<sub>1</sub> are selected from the group consisting of hydrogen and halogen.

40. An electrophotographic material comprising an electrically conductive support layer and a photoconductive insulating layer, the latter containing an organic colloid and a compound having the formula



50 in which R and R<sub>2</sub> are hydrogen and R<sub>1</sub> and R<sub>3</sub> are alkyl radicals.

41. An electrophotographic material comprising an electrically conductive support layer and a photoconductive insulating layer, the latter containing an organic colloid and a compound having the formula



60 in which R and R<sub>2</sub> are hydrogen and R<sub>1</sub> and R<sub>3</sub> are acyl radicals.

65 References Cited by the Examiner

UNITED STATES PATENTS

|           |       |                 |           |
|-----------|-------|-----------------|-----------|
| 1,730,505 | 10/29 | Hart            | 252—510   |
| 2,663,636 | 12/53 | Middleton       |           |
| 2,692,178 | 10/54 | Grandadam       | 96—1      |
| 2,765,304 | 10/56 | Siegrist et al. | 260—307 X |
| 2,800,559 | 7/57  | Ubbesolde       |           |
| 2,825,814 | 3/58  | Walkup          | 96—1 X    |

(Other references on following page)

## FOREIGN PATENTS

134,610 6/47 Australia.  
201,416 4/56 Australia.

## OTHER REFERENCES

Kallmann et al., Physical Review, vol. 97, No. 6, pages 1596-1610 (1955).  
Winslow et al., Journ. Amer. Chem. Soc., vol. 77, pages 4751-4756 (Sept. 1955).

Deribere, Applications Pratiques de la Luminescence, Dunod (1938), pages 151-152.

Zchodro, J. Chim. Phys., vol. 29, pages 59-64 (1929).

Petrikaln, Z. Phys. Chem., vol. 10B, pages 9-21 (1930).

5 Vartanian, Physiochimica, VRSS vol. XXII, No. 2, pages 201-224 (1947).

NORMAN G. TORCHIN, *Primary Examiner.*

PHILIP E. MANGAN, MILTON STERMAN, HAROLD  
10 N. BURSTEIN, *Examiners.*